

J. P. CROWLEY.

METHOD AND APPARATUS FOR DRAWING SHEET GLASS.

APPLICATION FILED JUNE 4, 1920.

1,394,283.

Patented Oct. 18, 1921.



Inventor

Joseph P. Crowley

By Whittmore, Hubbell & Whittmore

Attorneys

# UNITED STATES PATENT OFFICE.

JOSEPH P. CROWLEY, OF TOLEDO, OHIO, ASSIGNOR TO THE LIBBEY-OWENS SHEET GLASS COMPANY, OF TOLEDO, OHIO, A CORPORATION OF OHIO.

## METHOD AND APPARATUS FOR DRAWING SHEET-GLASS.

1,394,283.

Specification of Letters Patent. Patented Oct. 18, 1921.

Application filed June 4, 1920. Serial No. 386,440.

To all whom it may concern:

Be it known that I, JOSEPH P. CROWLEY, a citizen of the United States of America, residing at Toledo, in the county of Lucas and State of Ohio, have invented certain new and useful Improvements in Methods and Apparatus for Drawing Sheet-Glass, of which the following is a specification, reference being had therein to the accompanying drawings.

The invention relates to the manufacture of sheet glass by methods of that type in which the sheet is drawn from a plastic mass, the opposite surfaces thereof being cooled and the edge portions being engaged with driven rolls which maintain the full width of the sheet. In such drawing operation it is necessary to pass the drawn sheet around a bending roll to change the direction from vertical to horizontal and also to contact the lower surface of the sheet with supporting rolls and with a drawing table. This contact with the rolls sometimes produces a marring of the surface 26 of the glass which is injurious to the quality.

It is the object of the present invention to obtain a method of drawing glass in which there will be no contact which can produce a marring effect on either surface 30 of the sheet. The essential feature of the method is in forming the contacting surface of glass which has a much smoother surface than the most highly polished metal. More specifically, my improved method consists in holding the drawn sheet out of contact with marring surfaces by supporting it upon a second drawn sheet which is intermediate the same and the bending and supporting rolls.

40 In the drawing I have illustrated an apparatus for carrying out my improved method, this being shown in vertical longitudinal section.

As the general type of apparatus is well known, I shall not describe or illustrate the same in detail, but as shown, A is the drawing chamber at the base of which is the receptacle B containing the mass of glass from which the sheet is drawn. C and C' 45 are heated chambers above portions of the mass in the receptacle B and which are separated from an intermediate space by depending lip tiles D and D'. Adjacent to these tiles are the tempering shields E and E' and between these tempering shields

is arranged an apparatus for simultaneously drawing two parallel sheets.

This apparatus comprises pairs of knurled rolls F arranged for engagement with the opposite edge portions of each of the two 60 sheets, these rolls being driven at a suitable speed by a mechanism not shown. The sheets are drawn upward to a bending roll G and are then passed around this roll in contact with each other. The adjacent surfaces of the sheets are, however, sufficiently cooled before they come into contact to prevent adhesion. After passing the bending roll the two sheets still in contact, pass over idler and guide rolls H—I and then on 70 to the drawing table J which may be of any suitable construction. To hold the sheets separate until they engage the bending roll G, I preferably arrange a roll K therebetween which holds the lower portion of the 75 sheets in substantial parallelism and changes the direction of the sheet but comes in direct contact with the bending roll.

With the apparatus as described and which is provided with all the necessary 80 auxiliary devices used in the single sheet drawing apparatus of this type, the two sheets will be drawn simultaneously and at the completion of the operation are freely separable from each other. The upper sheet 85 having been held out of direct contact with either the bending roll, idler rolls or drawing table it will be of high quality and free from mars. On the other hand, the lower sheet which may be somewhat inferior in quality is nevertheless usable for purposes not requiring the highest quality.

What I claim as my invention is:

1. In the process for manufacturing sheet glass, the step of advancing the drawn sheet 90 free from injurious contacts by the interposition between the same and its supports, of a directly contacting surface of glass.

2. In the process for manufacturing sheet glass, the step of advancing the drawn sheet 100 free from injurious contacts by the interposition between the sheet and its supports, of a traveling surface of glass.

3. The process for manufacturing sheet glass, comprising the simultaneous drawing 105 of two sheets, the holding of one of said sheets from injurious contacts by directly contacting the same with the other sheet and separating the sheets from each other.

4. The process of manufacturing sheet 110

glass, comprising the simultaneous drawing of a plurality of sheets, having portions thereof in separable contact with each other.

5. The process of manufacturing sheet glass, comprising the simultaneous drawing of a plurality of sheets, passing said sheets about a bending roll in separable contact with each other, continuing the drawing in a plane while still in contact and finally 10 separating the sheets.

6. The process of manufacturing sheet glass, comprising the simultaneous drawing of a plurality of sheets separate from each other, maintaining said sheets separate until 15 the surfaces thereof are sufficiently cooled to prevent permanent adhesion and in then passing said sheets into contact with each other and maintaining them in contact during the remainder of the drawing operation.

16 7. An apparatus for the manufacture of sheet glass, comprising a receptacle for plastic glass, means for drawing a plurality of separate sheets from the surface

of the glass in said receptacle and common supporting means over which the several 25 sheets are passed in separable contact with each other.

8. An apparatus for the manufacture of sheet glass, comprising a receptacle for the plastic glass, means for drawing vertically 30 from the surface of the glass in said receptacle a plurality of separate sheets and a common bending roll about which said sheets are drawn in separable contact with each other.

35 9. An apparatus for the manufacture of sheet glass, the combination of a receptacle for plastic glass, means for drawing vertically from said receptacle a plurality of separate sheets of glass, a common bending 40 roll about which said sheets are drawn in separable contact with each other and a common drawing table for supporting said sheets while still in contact.

In testimony whereof I affix my signature. 45  
JOSEPH P. CROWLEY.